

Oct. 29, 1940.

B. GASPAR

2,219,304

COLORED PHOTOGRAPHIC MULTILAYER MATERIAL

Filed Dec. 3, 1938



Inventor

*Bela Gaspar*

*F. Gerald Foye*  
Attorney

## UNITED STATES PATENT OFFICE

2,219,304

## COLORED PHOTOGRAPHIC MULTILAYER MATERIAL

Béla Gáspár, Hollywood, Calif.

Application December 3, 1938, Serial No. 243,887  
In Great Britain December 9, 1937

4 Claims. (Cl. 95—2)

Light-sensitive multilayer materials are known, which are formed by superimposed silver halide layers colored in the three colors, yellow magenta, and blue-green for subtractive color photography in which material the yellow layer is sensitized to blue, the magenta layer to green, and the blue-green layer to red. The use of such a material has, however, certain disadvantages. If, for instance, the coloration of the layers is very intense, the actinic light is prevented from entering the layers and the silver image will not extend to the bottom of the layers. If thereafter the dyestuff is destroyed at the points of the silver deposit, the lower strata of the layers cannot be decolorised and pure white cannot be obtained.

In my U. S. Patent No. 1,985,344 dated December 25, 1934, I have pointed out that by sensitizing, for example, a yellow colored emulsion not to blue light, as in the material described above, but to red or green light or to that part of blue light which is not absorbed by the dyestuff in the layer, the requirement of intense coloration of the layers and the necessity of completely penetrating exposure can be satisfied. On the other hand, one might imagine that the coloration of the layers could be chosen weak enough, so that the exposure of the layer throughout its entire depth is possible even with light absorbed by the dyestuff. Such small dyestuff concentrations are suitable for images on a paper support but in this case prints in somewhat distorted colors are obtained. It has been found that in the case of paper prints on a material having low dyestuff concentration in layers sensitized to light absorbed by the color of the layer the defects of the prints are due to the fact that the light which acts on the layer throughout its depth cannot be prevented by the weak color of the layer from passing through the layer and entering the following layer. If this following layer is sensitive for the light, which should only act in the preceding layer, the part image extends over the two layers instead of being restricted to the first one, and the false colors of the print are the result. In order to avoid this inconvenience and in order to produce a light-sensitive material on a paper support which allows the printing of copies on paper from multicolor originals or part images, the second of two superposed layers is dyed not only with a dyestuff of a color complementary to the light to which this second layer is to be exposed but in addition with a dyestuff of the same color as the image forming dyestuff present in the first

layer. The additional dyestuff in the second layer, as distinguished from the image forming dyestuff in the upper layer is, however, removable by treating solutions which do not affect the image forming dyestuffs or which act on the image forming dyestuff only in a selective manner according to the exposure of the layer. 5

*Example.*—On to a paper support there are coated in superposition, a blue-green dyed emulsion sensitized to red light or one containing a panchromatic sensitizer; a magenta dyed orthochromatic emulsion or one containing a green sensitizer, and finally a yellow dyed blue-sensitive emulsion, as shown in the figure of the drawing. 10

The yellow dyed emulsion is the top layer and contains the dyestuff Xylenewalkgelb G (Schultz Farbstofftabellen, Leipzig 1932, 7th edition, volume 2, page 232) in the form of its calcium salt in a concentration of 0.45 g. per sq. in. Then follows the magenta layer which contains 0.3 g. per sq. m. of the dyestuff Tuchehtbrillantrot 2B (a dyestuff supplied by the Gesellschaft fuer Chemische Industrie in Basle and similar to the dyestuff Polarbrillantrot B described in Brunner, Analyse der Azofarbstoffe, Berlin 1929, page 113) in the form of its N-methyl-naphthoquinolinium salt, which may conveniently be formed by the action of a solution containing N-methyl-quino- 15 linium-methyl-sulphonate on the dyestuff. This layer is formed by an ordinary blue-sensitive emulsion to which a green-sensitizer has been added. The same layer further contains about 1.5 g. of the dyestuff 4,4'-methenyl-bis-[1-(p-sulphophenyl)-3-methyl-pyrazolone-5] described in 20 my application Ser. No. 240,860 filed November 16, 1938. This yellow dyestuff may be fixed in the layer in the form of its triphenyl guanidine salt. Behind the green sensitized layer containing the magenta dyestuff and the auxiliary yellow dyestuff a panchromatic or red sensitized emulsion dyed blue-green by 0.35 g. per sq. m. of the dyestuff Pontamine Sky Blue 5BX (Schultz Farbstofftabellen 1931, 7th edition, vol. 1, number 513) is arranged on the paper support of the 25 combined multi-layer material. The blue-green dyestuff may be fixed in the form of an insoluble salt, and this layer may further contain 1 g. per sq. m. of the dyestuff obtained from 1-(p-sulphophenyl)-3-methyl-pyrazolone-5 and  $\beta$ -anilino-acroleine-anil as described in Example 30 of my application Ser. No. 240,860 filed November 16, 1938, or of the sulphonic acid derived from methenyl - bis - oxythionaphthene (Beilstein, Handbuch der Organischen Chemie, 4th edi- 35 40 45 50 55

tion, 1934, supplement, volume XIX, page 713) or other decolorisable red dyestuff. The sulphonate derivative of methenyl-bis-oxythiophenol may be obtained by the sulphonation of this body with fuming sulphuric acid containing 20% sulphur trioxide.

In the specification the term "first" layer refers to that one of two superposed layers which is first illuminated by light and the term "second layer" refers to the following layer. The terms include the top layer and the middle layer in a three layer material as well as the middle layer and the rear layer. The image forming dyestuffs may be water soluble dyestuffs of low diffusion which 5 fastly dye the layer or insoluble salts of water, soluble dyestuffs or even insoluble dyes, such as insoluble oxy- or amino-azodyestuffs. The material may be exposed behind colored or black and white positive part images or behind a multi- 10 color master-positive of the additive or subtractive type. The auxiliary dyestuffs are decolorised after exposure of the three layer material preferably by a developer of alkaline reaction, and the image-forming dyestuffs are locally destroyed 15 after development of the silver images, for example, by an acid thiocarbamide solution or by a solution containing 5% hydrobromic acid. If necessary the silver is afterwards removed from 20 the dyestuff image thus obtained.

30 What is claimed is:

1. A multilayer light-sensitive material comprising a support, carrying a plurality of superposed silver halide emulsion layers sensitive to light of different colors, at least one of the layers 35 being dyed by a dye which is fast to ordinary photographic treating solutions but capable of being locally bleached in the presence of a metallic silver image and which absorbs light rays for which the layer is predominantly sensitized, the 40 one of said plurality of superposed light-sensitive layers arranged next behind said fast dyed layer being colored with a removable filter dye of substantially the same color as said fast dye, said filter dye being removable by an agent which 45 does not remove said fast dye.

2. A multilayer light-sensitive material comprising a support, carrying a plurality of superposed silver halide emulsion layers sensitive to light of different colors, at least one of the layers

being dyed by a dye which is fast to ordinary photographic treating solutions but capable of being locally bleached in the presence of a metallic silver image and which absorbs light rays for which the layer is predominantly sensitized, the 5 one of said plurality of superposed light-sensitive layers arranged next behind said fast dyed layer being colored with a filter dye which is of substantially the same color as said fast dye and is destroyable by a photographic developer which 10 does not remove said fast dye.

3. A multilayer light-sensitive material comprising a support, carrying a plurality of superposed silver halide emulsion layers sensitive to light of complementary colors, each of the layers being dyed by a dye which is fast to ordinary photographic treating solutions but capable of being locally bleached in the presence of a metallic silver image and which absorbs light rays for which the layer is predominantly sensitized, one 15 of said plurality of superposed light-sensitive layers arranged next behind another of said layers being colored with a filter dye which is substantially of the same color as the fast dye in said other colored layer and is destroyable by an alkaline photographic developer which does not remove the fast dye in any of said layers.

4. A multilayer light-sensitive material comprising a support, carrying a plurality of superposed silver halide emulsion layers sensitive to light of different colors, at least one of the layers being dyed by a dye which is fast to ordinary photographic treating solutions but capable of being locally bleached in the presence of a metallic silver image and which absorbs light rays for which the layer is predominantly sensitized, the one of said plurality of superposed light-sensitive layers arranged next behind said fast dyed layer being colored with a removable filter dye of substantially the same color as the fast dye in 30 said first mentioned layer and a dye which is fast to ordinary photographic treating solutions but capable of being locally bleached in the presence of a metallic silver image and which absorbs light 35 rays for which the layer is predominantly sensitized, said removable filter dye being removable by an agent which does not remove the fast dyes in 40 said layers.

BÉLA GÁSPÁR.